

## UNITED STATES PATENT OFFICE

2,067,308

## STAINLESS COPPER BASE ALLOYS

Richard A. Wilkins, Rome, N. Y., assignor to  
Revere Copper and Brass Incorporated, Rome,  
N. Y., a corporation of Maryland

No Drawing. Original application May 31, 1933,  
Serial No. 673,768. Divided and this applica-  
tion November 1, 1934, Serial No. 751,090

6 Claims. (Cl. 75—159)

This application is a division of my co-pending application Serial No. 673,768, filed May 31, 1933.

My invention, which relates to stainless copper base alloys, and has among its objects the production of alloys of this kind which may be readily worked into sheets and other forms by usual mill processes, will be best understood from the following description of several examples of the alloy compounded according to the invention, the scope of which latter will be more particularly pointed out in the appended claims.

Heretofore copper base alloys containing nickel and chromium have been employed in practice only for castings. For economic reasons it has been impractical to roll or otherwise mechanically work such prior alloys as they are brittle, difficult to work cold, and next to impossible to work hot.

Applicant has found that workable stainless copper base alloys can be produced by compounding copper, nickel and chromium in proper proportions particularly when suitable precautions are taken to secure solution of the chromium and to prevent deleterious secondary compounds. These alloys may be readily cold and hot rolled into sheets and may be otherwise attenuated while cold or hot by usual mill processes to produce various shapes.

The alloy may be compounded with or without zinc, but preferably with it except as herein-after mentioned, as its presence it has been found facilitates the working of the alloy particularly when it is to be annealed between the attenuating steps in the mill processes. Further, the alloy preferably is compounded with an additional constituent or constituents, herein-after for convenience in terminology referred to as "chromium incorporators", which will insure protecting the chromium from oxidation and insure its solution, and preferably also insure eliminating the effect on the nickel of any sulphur that may be present. In the absence of protecting the chromium from oxidation, the chromium when melted in or with cupro-nickel is liable to come off as a slag or be in the form of an oxide distributed throughout the alloy, and if material amounts of sulphur are present and are allowed to combine with the nickel the resulting nickel-sulphid may seriously interfere with the facility with which the alloy may be worked. It has been found that manganese will insure the solution of the chromium in the copper base alloy, and, as manganese has a greater affinity than chromium for oxygen and a greater

affinity than nickel for sulphur, any possibility of oxidation of the chromium and formation of nickel-sulphid is prevented effectively by use of this metal. The manganese-sulphid has no appreciable effect upon the workability of the alloy, and any excess of manganese, over that necessary to secure these results within the range of metals hereinafter stated, enters into solution and augments the effect of the nickel as a whitener for the alloy.

As a substitute for manganese as a so-called "chromium incorporator", small amounts of magnesium and tin may be employed. The magnesium will prevent any possibility of oxidation of the chromium and formation of nickel-sulphid, while the tin will insure the solution of the chromium. In employing magnesium precaution should be taken not to employ an amount thereof materially in excess of that necessary to take up the oxygen and sulphur, small amounts of magnesium in excess of this, say in the order of 0.25% uncombined metal, deleteriously affecting the physical properties of the alloy within the ranges of metals herein stated. When manganese with tin is employed as a substitute for manganese the zinc may be omitted, and in practice ordinarily is.

When desired the tensile strength of the alloy may be increased and controlled by addition of small amounts of vanadium, say from traces up to 0.1%, this metal also much improving the cold working properties of the alloy and its ductility and elongation.

The amount of nickel may be varied to vary the color of the alloy. With a high nickel content of about 18% a bright, clear white metal characteristic of the color of stainless steel is secured. By decreasing the nickel content to 10% and below alloys of warmer tones are obtained, with a suggestion of a rose or pinkish tint underlying the white, which warmer tones are desirable for architectural work. The nickel content should ordinarily not exceed approximately from 20 to 22%, as above these values the alloy becomes increasingly difficult to work. On the other hand, the nickel content should not ordinarily be less than approximately from 4 to 5%, as below these values the alloy loses its characteristic color and ceases to be stainless.

The copper content should be relatively high, and ordinarily not less than approximately 65% of the alloy, as with lower copper values the alloy becomes increasingly brittle and difficult to work. Further, the copper content should not exceed approximately 90% when zinc and man-

ganese are employed, or exceed approximately 93% when zinc is omitted and magnesium with tin is employed as a substitute for manganese.

Further, to secure the desirable properties of the alloy within the ranges of other constituents hereinafter mentioned, the sum of the copper and nickel should not be less than approximately 80%, or when zinc is present exceed approximately 95%, or in the absence of zinc exceed approximately 10 97%.

It has been found that the amount of chromium ordinarily should not exceed approximately 5% as values in excess of this make the alloy difficult to work, and ordinarily should not be less than approximately 0.5% to insure that the alloy is stainless. It has further been found, that to secure the desirable properties of the alloy within this range of chromium, the amount thereof should vary approximately linearly and inversely 15 with the amount of copper, satisfactory results ordinarily being secured when the amount of chromium is within plus or minus 25% of the value determined by this ratio, so long as it is not materially above the maximum or below the minimum values thereof of 5 and 0.5% respectively.

It has been found that under ordinary conditions amounts of manganese less than 0.25% will not insure satisfactory results, and that amounts in excess of 5% are likely to cause the alloy to 30 become brittle and refractory with the range of chromium above stated. Further, to secure best results, the amount of manganese should vary approximately linearly and directly with the amount of chromium, it ordinarily being satisfactory when the amount of manganese is within plus or minus 25% of the value determined by this ratio. When magnesium with tin is employed as a substitute for manganese, to prevent the presence of a deleterious excess of magnesium, over that necessary to prevent both oxidation of the chromium and formation of deleterious amounts of nickel-sulphid, the amount of magnesium should ordinarily not exceed approximately 5%, and, to insure satisfactory effects, should ordinarily not be less than approximately 0.25%, while within the range of chromium above stated the amount of tin should not exceed approximately 0.5% or be less than approximately 0.1%. To secure best results, the specific 45 amounts of magnesium and tin should, like the manganese, ordinarily vary approximately linearly and directly with the amount of chromium, satisfactory results ordinarily being secured when the amounts of magnesium and tin are within plus or minus 25% of the value determined by this ratio.

As hereinbefore mentioned, the zinc, which preferably is employed, particularly when manganese is used to facilitate incorporation of the 60 chromium, should not exceed approximately 20% of the alloy, as zinc values in excess of this tend to make the alloy brittle.

The general approximate formula for the basic copper, nickel, chromium alloys may be stated as 65 copper 65 to 93 parts, nickel 4 to 22 parts, and chromium 0.5 to 5 parts, with the sum of the copper and nickel between 80 and 97 parts. When zinc is added to these basic alloys, the general approximate formula becomes copper 65 to 93 parts, 70 nickel 4 to 22 parts, chromium 0.5 to 5 parts, and zinc the balance to make 100 parts, with the sum of the copper and nickel as before; and if the alloys contain vanadium the same may be substituted for an equal part of the zinc. When a 75 "chromium incorporator" is employed with these

basic copper, nickel chromium alloys, 0.25 to 5 parts manganese (or 0.25 to 5 parts magnesium plus 0.1 to 0.5 parts tin) may be employed. When both zinc and the "chromium incorporator" are employed with these basic copper, nickel, chromium alloys, which may be done if desired, the zinc should be largely substituted for part of the copper, in which case the general approximate formula for the alloys becomes copper 65 to 90%, nickel 5 to 22%, chromium 0.5 to 5%, manganese 0.25 to 5% (or magnesium 0.25 to 5% plus tin 0.1 to 0.5%), and zinc the balance, the sum of the copper and nickel being between 80 and 95%, any vanadium, employed being substituted for an equal part of the zinc. As has hereinbefore been mentioned, in all these cases the chromium within the range thereof stated preferably should vary approximately linearly and inversely with the amount of copper and the manganese; magnesium and tin within the ranges thereof stated preferably should vary approximately linearly and directly with the amount of chromium. Alloys consisting of copper 65 to 93 parts, nickel 4 to 22 parts, with the sum of the copper and nickel 80 to 97 parts, chromium 0.5 to 5 parts, and manganese 0.5 to 5 parts, have the following approximate percentage composition: copper 66.5 to 95.3%, nickel 3.6 to 25%, with the sum of the copper and nickel 89 to 99%, chromium 0.5 to 5.5%, and manganese 0.5 to 5.5%. 10 15 20 25 30

As suitable alloys for fabricating sheets for architectural purposes, the following give satisfactory results:

|          | Percent  |
|----------|----------|
| Copper   | 75       |
| Nickel   | 18       |
| Chromium | 0.5 to 1 |
| Zinc     | Balance  |

or the above alloys containing from 0.5 to 1% manganese substituted for an equal amount of the zinc, and in either case, if desired, small amounts of vanadium in the order of 0.01%.

As suitable alloys for fabricating sheets for automobile headlights, radiators, and the like, the following give satisfactory results:

|           | Percent      |
|-----------|--------------|
| Copper    | 68           |
| Nickel    | 19           |
| Chromium  | 3 to 3.5     |
| Manganese | 4            |
| Vanadium  | 0.02 to 0.03 |
| Zinc      | Balance      |

It has been found that excellent alloys satisfactory for ordinary purposes can be compounded according to the invention consisting of

|           | Percent       |
|-----------|---------------|
| Copper    | 65 to 93      |
| Nickel    | 8 to 18       |
| Chromium  | 1 to 4        |
| Tin       | 0.2 to 0.4    |
| Magnesium | 1 to 4        |
| Vanadium  | Traces to 0.1 |

an excellent alloy of this series consisting of

|           | Percent |
|-----------|---------|
| Copper    | 84      |
| Nickel    | 11      |
| Chromium  | 3.5     |
| Tin       | 0.25    |
| Magnesium | 1.4     |
| Vanadium  | Trace   |

As a suitable method of compounding the above alloys the copper and nickel may be melted together and the temperature of the melt

- raised to about 2300° F. The manganese may then be added in the form of a copper alloy rich in manganese, say one containing 25% manganese. The chromium may be added in the 5 form of a copper alloy rich in chromium, say one containing 10% chromium, and then the vanadium may be added in the same way. The zinc may be added in the form of brass to cool the melt to about 2000° F. just before pouring.
- 10 When the alloy contains tin the same may be added to the molten copper and nickel in the form of bronze scrap, after which the magnesium and chromium may be added, in the form of a copper alloy rich in both these metals, 15 shortly before pouring.

It will be understood that small proportions of other metals than those herein mentioned may be added to the alloy to give it special characteristics when they do not to a material 20 extent change the hereinbefore mentioned desirable physical and chemical properties of the alloy, and also that wide deviations may be made from the embodiments of the invention herein described without departing from the 25 spirit of the invention.

I claim

1. Stainless, hot and cold workable, white metal alloys containing copper 66.5 to 95.3%, nickel 3.6 to 25%, chromium 0.5 to 5.5%, manganese 0.5 to 5.5%, the sum of the copper and nickel being between 89 and 99%, the amount 30 of chromium varying roughly linearly and inversely with the amount of copper within the ranges of chromium and copper specified, the

copper and nickel constituting substantially the balance of the alloy with respect to the other elements specified.

2. Stainless hot and cold workable, white metal alloys containing copper 66.5 to 95.3%; 5 nickel 3.6 to 25%, chromium 0.5 to 5.5%, manganese 0.5 to 5.5%, the sum of the copper and nickel being between 89 and 99%, the amount of manganese varying roughly linearly and directly with the amount of chromium, the copper and nickel constituting substantially the balance of the alloy with respect to the other elements specified.

3. Stainless, hot and cold workable, white metal alloys containing copper 66.5 to 95.3% 15 nickel 3.6 to 25%, chromium 0.5 to 5.5%, manganese 0.5 to 5.5%, the sum of the copper and nickel being between 89 and 99%, the amount of chromium varying roughly linearly and inversely with the amount of copper within the 20 ranges of chromium and copper specified, and the amount of manganese varying roughly linearly and directly with the amount of chromium, the copper and nickel constituting substantially the balance of the alloy with respect 25 to the other elements specified.

4. The alloys according to claim 1 containing appreciable amounts up to 0.1% vanadium.

5. The alloys according to claim 2 containing 30 appreciable amounts up to 0.1% vanadium.

6. The alloys according to claim 3 containing appreciable amounts up to 0.1% vanadium.

RICHARD A. WILKINS.